# EUROPEAN PATENT SPECIFICATION

(11) **EP 4 235 714 B1**
(45) Date of publication and mention of the grant of the patent: **19.02.2025**
(21) Application number: 21886214.2
(22) Date of filing: 26.10.2021
(51) Int. Cl.: H01F 41/02, H01F 27/245

(54) **WOUND CORE, METHOD OF PRODUCING WOUND CORE AND WOUND CORE PRODUCTION DEVICE**
GEWICKELTER KERN, VERFAHREN ZUR HERSTELLUNG EINES GEWICKELTEN KERNS UND VORRICHTUNG ZUR HERSTELLUNG EINES GEWICKELTEN KERNS
NOYAU DE FER ENROULÉ, PROCÉDÉ DE FABRICATION DE NOYAU DE FER ENROULÉ ET APPAREIL DE FABRICATION DE NOYAU DE FER ENROULÉ

(30) Priority: 26.10.2020 JP 2020178561
(43) Date of publication of application: 30.08.2023
(73) Proprietor: NIPPON STEEL CORPORATION, Chiyoda-ku Tokyo 100-8071 (JP)
(72) Inventor: IWAKI, Masataka, Tokyo 100-8071 (JP); MIZUMURA, Takahito, Tokyo 100-8071 (JP); MOGI, Hisashi, Tokyo 100-8071 (JP)
(74) Representative: Vossius & Partner Patentanwälte Rechtsanwälte mbB
(86) International application number: PCT/JP2021/039519
(87) International publication number: WO 2022/092096

(56) References cited:
- WO-A1-2018/131613
- WO-A1-2018/131613
- JP-A- 2018 148 036
- JP-A- 2018 148 036
- JP-A- 2021 163 942

## Description

### [Technical Field]

The present invention relates to a wound core, a method of producing a wound core, and a wound core production device. Priority is claimed on Japanese Patent Application No. 2020-178561, filed October 26, 2020.

### [Background Art]

Transformer iron cores include stacked iron cores and wound cores. Among these, the wound core is generally produced by stacking grain-oriented electrical steel sheets in layers, winding them in a donut shape (wound shape), and then pressing the wound body to mold it into substantially a rectangular shape (in this specification, a wound core produced in this manner may be referred to as a trunk core). According to this molding process, mechanical processing strain (plastic deformation strain) is applied to all of the grain-oriented electrical steel sheets, and the processing strain is a factor that greatly deteriorates the iron loss of the grain-oriented electrical steel sheet so that it is necessary to perform strain relief annealing.

On the other hand, as another method of producing a wound core, techniques such as those found in Patent Documents 1 to 3 in which portions of steel sheets that become corner portions of a wound core are bent in advance so that a relatively small bending area with a radius of curvature of 3 mm or less is formed and the bent steel sheets are laminated to form a wound core are disclosed (in this specification, the wound core produced in this manner may be referred to as Unicore (registered trademark)). According to this production method, a conventional large-scale pressing process is not required, the steel sheet is precisely bent to maintain the shape of the iron core, and processing strain is concentrated only in the bent portion (comer) so that it is possible to omit strain removal according to the above annealing process, and its industrial advantages are great and its application is progressing.

### [Citation List]

### [Patent Document]

[Patent Document 1]
   Japanese Unexamined Patent Application, First Publication No. 2005-286169
[Patent Document 2]
   Japanese Patent No. 6224468
[Patent Document 3]
   Japanese Unexamined Patent Application, First Publication No. 2018-148036

### [Summary of the Invention]

### [Problems to be Solved by the Invention]

Incidentally, in the production of Unicore, although the range of plastic deformation strain (processing strain) introduced according to bending of a steel sheet is limited, along with bending (introduction of plastic strain), the surface shape of the bent portion also changes into an undulating shape and becomes rough, and as a result, the frictional force between the steel sheets that overlap each other increases, and it cannot be denied that noise caused by vibration during excitation increases (noise properties significantly deteriorate).

The present invention has been made in view of the above circumstances, and an object of the present invention is to provide a wound core, a method of producing a wound core, and a wound core production device through which it is possible to reduce noise caused by plastic deformation strain introduced according to bending of a steel sheet.

### [Means for Solving the Problem]

In order to achieve the above object, the present invention provides a wound core including a portion in which grain-oriented electrical steel sheets in which planar portions and bent portions are alternately continuous in a longitudinal direction are stacked in a sheet thickness direction and formed by stacking the grain-oriented electrical steel sheets that have been individually bent in layers and assembled into a wound shape, wherein, when an average height of a roughness curve element in a width direction intersecting the longitudinal direction forming a surface of the bent portion of the grain-oriented electrical steel sheet is Ra(b), and an average height of the roughness curve element in the width direction forming a surface of the planar portion of the grain-oriented electrical steel sheet is Ra(s), the relationship of 1.00<Ra(b)/Ra(s)≤5.00 is satisfied.

The wound core having the above configuration of the present invention is formed by stacking the grain-oriented electrical steel sheets that have been individually bent in layers and assembled into a wound shape (a so-called Unicore in which strain relief annealing can be omitted), and when bending is performed while tensile stress is applied to the entire end surface (C cross section) of the steel sheet to be bent in the longitudinal (rolling) direction (L direction), the average height of the roughness curve element in the width direction intersecting the longitudinal direction forming a surface (outline) of the bent portion of the grain-oriented electrical steel sheet is Ra(b), and the average height of the roughness curve element in the width direction forming a surface (outline) of the planar portion of the grain-oriented electrical steel sheet is Ra(s), the relationship of 1.00<Ra(b)/Ra(s)≤5.00 is satisfied. Here, the surface of the bent portion and the surface of the planar portion refer to the surface (the outer surface of the bent portion and the planar portion) facing the outside of the wound core. Here, Ra(b) and Ra(s) both are the average height Rc of the roughness curve element defined in JIS B0601 (2013).

As described above, in the production of Unicore, due to plastic strain introduced into the grain-oriented electrical steel sheet according to bending, the frictional force between the steel sheets overlapping each other increases, and accordingly, there is a problem of noise caused by vibration during excitation increasing. Thus, the inventors focused on the fact that, when the grain-oriented electrical steel sheet is bent while applying tensile stress in the longitudinal direction (the rolling direction), the roughness outside the bent region (bent portion) of the grain-oriented electrical steel sheet is reduced (smoothened), and found that, when bending is performed while applying tensile stress to the steel sheet in the longitudinal direction during bending, the relationship of 1.00<Ra(b)/Ra(s)≤5.00 is satisfied (or the average height Ra of the roughness curve element inside and outside the bent region of the grain-oriented electrical steel sheet is controlled), noise caused by plastic deformation strain is reduced. This is understood as follows: when the grain-oriented electrical steel sheet is bent while applying tension in the longitudinal direction, a proportion of plastic strain due to tension in the deformation strain introduced into the bent region increases (the ratio of compress strain decreases with respect to the ratio of tension strain), and the average height (Ra(b)) of the roughness curve element outside the bent region of the grain-oriented electrical steel sheet is reduced (smoothened), and accordingly, the frictional force between the steel sheets overlapping each other in a laminated state is reduced and noise caused by vibration during excitation (particularly, in the bent region) is reduced.

Here, the average height of the roughness curve element is determined according to Japanese Industrial Standard JIS B 0601 (2013). In addition, in the above configuration, the bent portion of the grain-oriented electrical steel sheet preferably has a radius of curvature of 1 mm or more and 5 mm or less. Here, the radius of curvature of the bent portion is the inner radius of curvature of the bent portion in a side view.

In addition, the present invention provides a method of producing a wound core including a bending process in which grain-oriented electrical steel sheets are individually bent and an assembling process in which the bent grain-oriented electrical steel sheets are stacked in layers and assembled into a wound shape to form a wound core having a wound shape including a portion in which grain-oriented electrical steel sheets in which planar portions and bent portions are alternately continuous in a longitudinal direction are stacked in a sheet thickness direction, wherein, in the bending process, the grain-oriented electrical steel sheet is bent while a tensile stress in a range of 4 MPa or more and 16 MPa or less is applied to the grain-oriented electrical steel sheet in the longitudinal direction.

In addition, the present invention provides a wound core production device including a bending unit that individually bends grain-oriented electrical steel sheets and an assembly unit that stacks the bent grain-oriented electrical steel sheets in layers and assembles them into a wound shape to form a wound core having a wound shape including a portion in which grain-oriented electrical steel sheets in which planar portions and bent portions are alternately continuous in a longitudinal direction are stacked in a sheet thickness direction, wherein the bending unit bends the grain-oriented electrical steel sheet while applying a tensile stress in a range of 4 MPa or more and 16 MPa or less to the grain-oriented electrical steel sheet in the longitudinal direction.

In the production method and production device having the above configuration, when the grain-oriented electrical steel sheets are individually bent, the grain-oriented electrical steel sheet is bent while a tensile stress in a range of 4 MPa or more and 16 MPa or less is applied to the grain-oriented electrical steel sheet in the longitudinal direction (the rolling direction) of the steel sheet. The steel sheet is bent while applying tensile stress under such conditions, and as a result, the relationship of 1.00<Ra(b)/Ra(s)≤5.00 is satisfied, and the same operational effects as in the above wound core can be obtained. That is, due to the influence of tensile stress applied in the longitudinal direction, the average height (Ra(b)) of the roughness curve element outside the bent region of the grain-oriented electrical steel sheet after bending is reduced (smoothened), and accordingly, the frictional force between the steel sheets overlapping each other in a laminated state is reduced and noise caused by vibration during excitation (particularly, in the bent region) is reduced (noise properties are improved). In addition, in the production method and production device having the above configuration, in the bending, the grain-oriented electrical steel sheet is preferably bent at a strain rate of 5 mm/sec or more and 100 mm/sec or less while applying a tensile stress in a range of 4 MPa or more and 16 MPa or less to the grain-oriented electrical steel sheet in the longitudinal direction. In addition, in the bending, the grain-oriented electrical steel sheet is preferably bent so that the radius of curvature of the bent portion of the grain-oriented electrical steel sheet is 1 mm or more and 5 mm or less.

### [Effects of the Invention]

According to the present invention, the grain-oriented electrical steel sheet is bent while applying tension in the longitudinal direction and the relationship of 1.00<Ra(b)/Ra(s)≤5.00 is satisfied so that the roughness outside the bent region (bent portion) of the grain-oriented electrical steel sheet after bending is reduce, and accordingly, the frictional force between steel sheets that overlap each other in a laminated state is reduced and noise caused by vibration during excitation is reduced.

### [Brief Description of Drawings]

FIG. 1 is a perspective view schematically showing a wound core according to one embodiment of the present invention.
FIG. 2 is a side view of the wound core shown in the embodiment of FIG. 1.
FIG. 3 is a side view schematically showing a wound core according to another embodiment of the present invention.
FIG. 4 is a side view schematically showing an example of a single-layer grain-oriented electrical steel sheet constituting a wound core.
FIG. 5 is a side view schematically showing another example of the single-layer grain-oriented electrical steel sheet constituting the wound core.
FIG. 6 is a side view schematically showing an example of a bent portion of the grain-oriented electrical steel sheet constituting the wound core of the present invention.
FIG. 7 is a diagram showing an example of a method of measuring an average height Ra(b) of a roughness curve element in a width direction forming a surface of a bent portion and an average height Ra(s) of a roughness curve element in a width direction forming a surface of a planar portion.
FIG. 8 is a schematic perspective view showing an example of a device for realizing bending in which a steel sheet is bent while applying tensile stress to a steel sheet portion to be bent in a longitudinal direction.
FIG. 9 is a block diagram schematically showing a configuration of a device for producing a Unicore type wound core including grain-oriented electrical steel sheets with elastic deformation on planar portions.
FIG. 10 is a schematic view showing sizes of a wound core produced when properties are evaluated.

### [Embodiment(s) for implementing the Invention]

Hereinafter, a wound core according to one embodiment of the present invention will be described in detail in order. However, the present invention is not limited to only the configuration disclosed in the present embodiment, and can be variously modified without departing from the gist of the present invention. Here, lower limit values and upper limit values are included in the numerical value limiting ranges described below. Numerical values indicated by "more than" or "less than" are not included in these numerical value ranges. In addition, unless otherwise specified, "%" relating to the chemical composition means "mass%."

In addition, terms such as "parallel," "perpendicular," "identical," and "right angle" and length and angle values used in this specification to specify shapes, geometric conditions and their extents are not bound by strict meanings, and should be interpreted to include the extent to which similar functions can be expected.

In addition, in this specification, "grain-oriented electrical steel sheet" may be simply described as "steel sheet" or "electrical steel sheet," and "wound core" may be simply described as "iron core."

The wound core according to one embodiment of the present invention is a wound core including a substantially rectangular wound core main body in a side view, and the wound core main body includes a portion in which grain-oriented electrical steel sheets in which planar portions and bent portions are alternately continuous in the longitudinal direction are stacked in a sheet thickness direction and has a substantially polygonal laminated structure in a side view. The inner radius of curvature r of the bent portion in a side view is, for example, 1 mm or more and 5 mm or less. As an example, the grain-oriented electrical steel sheet has a chemical composition containing, in mass%, Si: 2.0 to 7.0%, with the remainder being Fe and impurities, and has a texture oriented in the Goss orientation. As the grain-oriented electrical steel sheet, for example, a grain-oriented electromagnetic steel band described in JIS C 2553: 2019 can be used.

Next, the shapes of the wound core and the grain-oriented electrical steel sheet according to one embodiment of the present invention will be described in detail. The shapes themselves of the wound core and the grain-oriented electrical steel sheet described here are not particularly new, and merely correspond to the shapes of known wound cores and grain-oriented electrical steel sheets.

FIG. 1 is a perspective view schematically showing a wound core according to one embodiment, FIG. 2 is a side view of the wound core shown in the embodiment of FIG. 1. In addition, FIG. 3 is a side view schematically showing another embodiment of the wound core.

Here, in the present invention, the side view is a view of the long-shaped grain-oriented electrical steel sheet constituting the wound core in the width direction (Y-axis direction in FIG. 1). The side view is a view showing a shape visible from the side (a view in the Y-axis direction in FIG. 1).

A wound core 10 according to one embodiment of the present invention includes a substantially polygonal wound core main body in a side view. The wound core main body 10 has a substantially rectangular laminated structure in a side view in which grain-oriented electrical steel sheets 1 are stacked in a sheet thickness direction. The wound core main body 10 may be used as a wound core without change, or may include, as necessary, for example, a known fastener such as a binding band for integrally fixing a plurality of stacked grain-oriented electrical steel sheets.

In the present embodiment, the iron core length of the wound core main body 10 is not particularly limited. If the number of bent portions 5 is the same, even if the iron core length of the wound core main body 10 changes, the volume of the bent portion 5 is constant so that the iron loss generated in the bent portion is constant. If the iron core length is longer, the volume ratio of the bent portion 5 to the wound core main body 10 is smaller and the influence on iron loss deterioration is also small. Therefore, a longer iron core length of the wound core main body 10 is preferable. The iron core length of the wound core main body 10 is preferably 1.5 m or more and more preferably 1.7 m or more. Here, in the present invention, the iron core length of the wound core main body 10 is the circumferential length at the central point in the laminating direction of the wound core main body 10 in a side view.

Such a wound core can be suitably used for any conventionally known application.

The iron core according to the present embodiment has substantially a polygonal shape in a side view. In the description using the following drawings, for simplicity of illustration and description, a substantially rectangular (square) iron core, which is a general shape, will be described, but iron cores having various shapes can be produced depending on the angle and number of bent portions 5 and the length of the planar portion 4. For example, if the angles of all the bent portions 5 are 45° and the lengths of the planar portions 4 are equal, the side view is octagonal. In addition, if the angle is 60°, there are six bent portions 5, and the lengths of the planar portions 4 are equal, the side view is hexagonal.

As shown in FIG. 1 and FIG. 2, the wound core main body 10 includes a portion in which the grain-oriented electrical steel sheets 1 in which the planar portions 4 and 4a and the bent portions 5 are alternately continuous in the longitudinal direction are stacked in a sheet thickness direction and has a substantially rectangular laminated structure 2 having a hollow portion 15 in a side view. A corner portion 3 including the bent portion 5 has two or more bent portions 5 having a curved shape in a side view, and the sum of the bent angles of the bent portions 5 present in one corner portion 3 is, for example, 90°. The corner portion 3 has a planar portion 4a shorter than the planar portion 4 between the adjacent bent portions 5 and 5. Therefore, the corner portion 3 has a form including two or more bent portions 5 and one or more planar portions 4a. Here, in the embodiment of FIG. 2, one bent portion 5 has an angle of 45°. In the embodiment of FIG. 3, one bent portion 5 has an angle of 30°.

As shown in these examples, the wound core of the present embodiment can be formed with bent portions having various angles, but in order to minimize the occurrence of distortion due to deformation during processing and minimize the iron loss, the bent angle <p (ϕ1, <p2, <p3) of the bent portion 5 is preferably 60° or less and more preferably 45° or less. The bent angle <p of the bent portion of one iron core can be arbitrarily formed. For example, ϕ1=60° and ϕ2=30° can be set but it is preferable that folding angles (bent angles) be equal in consideration of production efficiency.

The bent portion 5 will be described in more detail with reference to FIG. 6. FIG. 6 is a diagram schematically showing an example of the bent portion (curved portion) 5 of the grain-oriented electrical steel sheet 1. The bent angle of the bent portion 5 is the angle difference occurring between the rear straight portion and the front straight portion in the bending direction at the bent portion 5 of the grain-oriented electrical steel sheet 1, and is expressed, on the outer surface of the grain-oriented electrical steel sheet 1, as an angle ϕ that is a supplementary angle of the angle formed by two virtual lines Lb-elongation1 and Lb-elongation2 obtained by extending the straight portions that are surfaces of the planar portions 4 and 4a on both sides across the bent portion 5. In this case, the point at which the extended straight line separates from the surface of the steel sheet is the boundary between the planar portion 4 and the bent portion 5 on the outer surface of the steel sheet, which is the point F and the point G in FIG. 6.

In addition, straight lines perpendicular to the outer surface of the steel sheet extend from the point F and the point G and intersections with the inner surface of the steel sheet are the point E and the point D. The point E and the point D are the boundaries between the planar portion 4 and the bent portion 5 on the inner surface of the steel sheet.

Here, in the present invention, the bent portion 5 is a portion of the grain-oriented electrical steel sheet 1 surrounded by the point D, the point E, the point F, and the point G in a side view of the grain-oriented electrical steel sheet 1. In FIG. 6, the surface of the steel sheet between the point D and the point E, that is, the inner surface of the bent portion 5, is indicated by La, and the surface of the steel sheet between the point F and the point G, that is, the outer surface of the bent portion 5, is indicated by L,b.

In addition, this drawing shows the inner radius of curvature r of the bent portion 5 in a side view. The radius of curvature r of the bent portion 5 is obtained by approximating the above La with a circular arc passing through the point E and the point D. A smaller radius of curvature r indicates a sharper curvature of the curved portion of the bent portion 5, and a larger radius of curvature r indicates a gentler curvature of the curved portion of the bent portion 5.

In the wound core of the present invention, the radius of curvature r at each bent portion 5 of the grain-oriented electrical steel sheets 1 laminated in the sheet thickness direction may vary to some extent. This variation may be a variation due to molding accuracy, and it is conceivable that an unintended variation may occur due to handling during lamination. Such an unintended error can be minimized to about 0.3 mm or less in current general industrial production. If such a variation is large, a representative value can be obtained by measuring the curvature radii of a sufficiently large number of steel sheets and averaging them. In addition, it is conceivable to change it intentionally for some reason, and the present invention does not exclude such a form.

Here, the method of measuring the radius of curvature r of the bent portion 5 is not particularly limited, and for example, the radius of curvature r can be measured by performing observation using a commercially available microscope (Nikon ECLIPSE LV150) at a magnification of 200. Specifically, the curvature center point A is obtained from the observation result, and for a method of obtaining this, for example, if the intersection of the line segment EF and the line segment DG extended inward on the side opposite to the point B is defined as A, the magnitude of the radius of curvature r corresponds to the length of the line segment AC*. Here, when the point A and the point B are connected by a straight line, the intersection on a circular arc DE inside the bent portion of the steel sheet is C*.

FIG. 4 and FIG. 5 are diagrams schematically showing an example of a single-layer grain-oriented electrical steel sheet 1 in a wound core main body. The grain-oriented electrical steel sheet 1 used in the examples of FIG. 4 and FIG. 5 is bent to realize a Unicore type wound core, and includes two or more bent portions 5 and the planar portion 4, and forms a substantially polygonal ring in a side view via a joining part 6 (gap) that is an end surface of one or more grain-oriented electrical steel sheets 1 in the longitudinal direction.

In the present embodiment, the entire wound core main body 10 may have a substantially polygonal laminated structure in a side view. As shown in the example of FIG. 4, one grain-oriented electrical steel sheet may form one layer of the wound core main body 10 via one joining part 6 (one grain-oriented electrical steel sheet is connected via one joining part 6 for each roll), and as shown in the example of FIG. 5, one grain-oriented electrical steel sheet 1 may form about half the circumference of the wound core, and two grain-oriented electrical steel sheets 1 may form one layer of the wound core main body via two joining parts 6 (two grain-oriented electrical steel sheets are connected to each other via two joining parts 6 for each roll).

The sheet thickness of the grain-oriented electrical steel sheet 1 used in the present embodiment is not particularly limited, and may be appropriately selected according to applications and the like, but is generally within a range of 0.15 mm to 0.35 mm and preferably in a range of 0.18 mm to 0.23 mm.

In addition, the method of producing the grain-oriented electrical steel sheet 1 is not particularly limited, and a conventionally known method of producing a grain-oriented electrical steel sheet can be appropriately selected. Specific examples of a preferable production method include, for example, a method in which a slab containing 0.04 to 0.1 mass% of C, with the remainder being the chemical composition of the grain-oriented electrical steel sheet, is heated to 1,000°C or higher and hot-rolled sheet annealing is then performed as necessary, and a cold-rolled steel sheet is then obtained by cold-rolling once, twice or more with intermediate annealing, the cold-rolled steel sheet is heated, decarburized and annealed, for example, at 700 to 900°C in a wet hydrogeninert gas atmosphere, and as necessary, nitridation annealing is additionally performed, an annealing separator is applied, finish annealing is then performed at about 1,000°C, and an insulation coating is formed at about 900°C. In addition, after that, a coating or the like for adjusting the dynamic friction coefficient may be implemented.

In addition, generally, the effects of the present invention can be obtained even with a steel sheet that has been subjected to a treatment called "magnetic domain control" using strain, grooves or the like in the steel sheet producing process by a known method.

In addition, in the present embodiment, the wound core 10 composed of the grain-oriented electrical steel sheet 1 having the above form is formed by stacking the grain-oriented electrical steel sheets 1 that have been individually bent in layers and assembled into a wound shape, and a plurality of grain-oriented electrical steel sheets 1 are connected to each other via at least one joining part 6 for each roll, but during individual bending, bending is performed while tensile stress is applied to the entire end surface (C cross section) of the steel sheet to be bent in the longitudinal direction, and when the average height of the roughness curve element in the width direction (Y-axis direction in FIG. 1) intersecting the longitudinal direction (the rolling direction L in FIG. 7) forming the surface (outline) of the bent portion 5 of the grain-oriented electrical steel sheet is Ra(b) and the average height of the roughness curve element in the width direction forming the surface (outline) of the planar portion 4 (4a) of the grain-oriented electrical steel sheet 1 is Ra(s), the relationship of 1.00<Ra(b)/Ra(s)≤5.00 is satisfied. In addition, in this case, the above radius of curvature (the inner radius of curvature of the bent portion 5 in a side view) r of the bent portion 5 is preferably 1 mm or more and 5 mm or less. When the radius of curvature r is set to 1 mm or more and 5 mm or less, it is possible to further reduce noise caused by vibration during excitation.

Here, regarding the average height Ra(b) of the roughness curve element in the width direction forming the surface of the bent portion 5 and the average height Ra(s) of the roughness curve element in the width direction forming the surface of the planar portion 4 (4a), for example, using a digital microscope (VHX-7000, commercially available from Keyence Corporation), average values are obtained by performing measurement at 10 fields of view at the bent portion 5 and the planar portion 4 (4a). Specifically, for example, a part of the grain-oriented electrical steel sheet 1 constituting the wound core is sheared and cut out as indicated by a dashed line in FIG. 7(a), and a cut steel sheet 1A including one corner portion 3 and planar portions 4 on both sides thereof as shown in FIG. 7(b) is obtained. During cutting, it is desirable to cut the planar portion 4 (4a) so that the bent portion 5 is not crushed. Here, regarding the cut steel sheet 1A, using the digital microscope, the outer surface of the planar portion 4 (4a) and the outer surface (Lb) of the bent portion 5 of the grain-oriented electrical steel sheet 1 facing the outside of the wound core are measured. Regarding the measurement position, it is desirable to perform measurement at the center of the steel sheet width (refer to measurement positions P and Q in FIG. 7(b)) far from the end surface of the steel sheet 1A. Here, as shown in FIG. 7(c), the bent portion 5, that is, a portion of the grain-oriented electrical steel sheet 1 surrounded by the point D, the point E, the point F, and the point G in FIG. 6, that is, in FIG. 7(c) showing a plane extending in a width direction C and a longitudinal direction L, an outer surface (Lb) portion surrounded by the point F, the point F,' the point G, and the point G' is scanned from above using the digital microscope in the width direction C as indicated by a dashed arrow, and Ra(b) is measured. Here, if necessary, the bent portion 5 to be measured may be marked in advance with a marker or the like. Similarly, regarding the planar portion 4 (4a), the outer surface portion is scanned from above using the digital microscope in the width direction C as indicated by a dashed arrow, and Ra(s) is measured. The planar portion 4 (4a) may be separately collected from the planar portion 4 (4a) of the same iron core or may be collected from a hoop left over after the iron core is produced. In any case, a steel sheet that is not plastically deformed may be used. For example, regarding the field of view for measurement, for example, the magnification is set to 200 so that the width of one field of view shown in FIG. 7(c) is 500 µm×500 µm. The average heights Ra(s) and Ra(b) of the roughness curve element are measured according to JIS B 0601

(2013). When the average height of the roughness curve elements is measured using a digital microscope, the cutoff value λs=0 µm and the cutoff value λc=0 mm, and vibration correction may be performed for measurement. The measurement magnification is preferably 100 or more and more preferably 500 to 700. Then, such measurement is performed on, for example, 10 cut steel sheets 1A, and average values thereof are defined as Ra(b) and Ra(s). Here, Ra(b) is preferably 0.5 µm to 4.0 µm. Ra(b) is more preferably 0.6 to 3.9 µm. In addition, Ra(s) is preferably 0.5 µm to 1.0 µm. Ra(s) is more preferably 0.6 µm to 0.8 µm.

In addition, bending performed to satisfy the relationship of 1.00<Ra(b)/Ra(s)≤5.00, that is, bending performed while applying tensile stress to the entire end surface (C cross section) of the steel sheet to be bent in the longitudinal direction L is performed by, for example, a bending unit 71 including a device 50 as shown in FIG. 8. The device 50 shown in FIG. 8 includes a steel sheet holding unit 52 that holds and fixes one side portion 1a of the grain-oriented electrical steel sheet 1, for example, in a holding state, and a bending mechanism 54 for performing bending in a direction Z perpendicular to the longitudinal direction L and the width direction C while holding other side end 1b of the grain-oriented electrical steel sheet 1 to be bent and applying tensile stress to the end surface of the other side end 1b in the longitudinal direction L. Specifically, the bending mechanism 54 includes a holding portion 62 that holds the other side end 1b of the grain-oriented electrical steel sheet 1, for example, in the direction Z perpendicular to the longitudinal direction L and the width direction C in a clamping manner, a tensile stress applying unit 63 that is provided on one side of the holding portion 62 in the longitudinal direction L and applies a tensile stress in a range of 4 MPa or more and 16 MPa or less to the other side end 1b of the grain-oriented electrical steel sheet 1 held by the holding portion 62 in the longitudinal direction L, and a bent portion forming portion 59 that presses down the holding portion 62 in the Z direction, bends the other side end 1b of the grain-oriented electrical steel sheet 1 held by the holding portion 62, for example, at a strain rate of 5 mm/sec or more and 100 mm/sec or less, and forms the bent portion 5. The tensile stress applying unit 63 can control tensile stress by a load meter 56 using a spring 55 and can set a load by a handle 57. In addition, the bent portion forming portion 59 includes a servo motor 58, a pump 60 that is driven by the servo motor 58, and an elevating portion 61 that is connected to the upper end of the holding portion 62, and the holding portion 62 can be moved in the Z direction by raising and lowering the elevating portion 61 with the pressure generated by the pump 60.

FIG. 9 schematically shows a production device 70 for a Unicore type wound core, and the production device 70 includes the bending unit 71 including the above device 50 for individual bending the grain-oriented electrical steel sheet 1, and stacks the bent grain-oriented electrical steel sheets 1 in layers and assembles them into a wound shape to form a wound core having a wound shape including a portion in which the grain-oriented electrical steel sheets 1 in which the planar portions 4 and the bent portions 5 are alternately continuous in the longitudinal direction are stacked in a sheet thickness direction. In this case, it may further include an assembly unit 72 that stacks the bent grain-oriented electrical steel sheets 1 in layers and assembles them into a wound shape.

The grain-oriented electrical steel sheets 1 are a fed at a predetermined conveying speed from a steel sheet supply unit 90 that holds a hoop member formed by winding the grain-oriented electrical steel sheet 1 in a roll shape and supplied to the bending unit 71. The grain-oriented electrical steel sheets 1 supplied in this manner are appropriately cut to an appropriate size in the bending unit 71 and subjected to bending in which a small number of sheets are individually bent such as one sheet at a time (bending process). In this bending, as described above, while a tensile stress in a range of 4 MPa or more and 16 MPa or less is applied to the grain-oriented electrical steel sheet 1 in the longitudinal direction L, the grain-oriented electrical steel sheet 1 is bent, for example, at a strain rate of 5 mm/sec or more and 100 mm/sec or less to form the bent portion 5. When a tensile stress in a range of 4 MPa or more and 16 MPa or less is applied to the grain-oriented electrical steel sheet 1, 1.00<Ra(b)/Ra(s)≤5.00 can be satisfied. In addition, in the bending process, it is preferable to bend the grain-oriented electrical steel sheet 1 so that the radius of curvature of the bent portion is 1 mm or more and 5 mm or less. In the grain-oriented electrical steel sheet 1 obtained in this manner, since the radius of curvature of the bent portion 5 caused by bending is very small, the processing strain applied to the grain-oriented electrical steel sheet 1 by bending is very small. In this manner, while the density of the processing strain is expected to increase, if the volume influenced by the processing strain can be reduced, the annealing process can be omitted. In addition, the grain-oriented electrical steel sheets 1 cut and bent in this manner are stacked in layers and assembled into a wound shape, for example, by the assembly unit 72, to form a wound core (assembling process).

Next, data verifying that noise is minimized with the wound core 10 having the above configuration according to the present embodiment is shown below.

The inventors produced iron cores a to f having shapes shown in Table 1 and FIG. 10 using respective steel sheets as materials when acquiring the verification data.

Here, L1 is parallel to the X-axis direction and is a distance between parallel grain-oriented electrical steel sheets 1 on the innermost periphery of the wound core in a flat cross section including the center CL (a distance between inner side planar portions). L2 is parallel to the Z-axis direction and is a distance between parallel grain-oriented electrical steel sheets 1 on the innermost periphery of the wound core in a vertical cross section including the center CL (a distance between inner side planar portions). L3 is parallel to the X-axis direction and is a lamination thickness of the wound core in a flat cross section including the center CL (a thickness in the laminating direction). L4 is parallel to the X-axis direction and is a width of the laminated steel sheets of the wound core in a flat cross section including the center CL. L5 is a distance between planar portions that are adjacent to each other in the innermost portion of the wound core and arranged to form a right angle together (a distance between bent portions). In other words, L5 is a length of the planar portion 4a in the longitudinal direction having the shortest length among the planar portions 4 and 4a of the grain-oriented electrical steel sheets on the innermost periphery, r is the radius of curvature of the bent portion 5 on the inner side of the wound core, and ϕ is the bent angle of the bent portion 5 of the wound core. The cores Nos. a to f of the substantially rectangular iron cores in Table 1 have a structure in which a planar portion with an inner side planar portion distance of L1 is divided at approximately in the center of the distance L1 and two iron cores having "substantially a U-shape" are connected.

Here, the iron core of the core No. e is conventionally used as a general wound core, and is a so-called trunk core type wound core produced by a method of shearing a steel sheet, winding it into a cylindrical shape, then pressing the cylindrical laminated body without change so that the corner portion has a constant curvature, and forming it into substantially a rectangular shape. Therefore, the radius of curvature of the bent portion 5 varies greatly depending on the lamination position of the steel sheet. Regarding the iron core of the core No. e, in Table 1, * indicates that r increases toward the outside, r=5 mm at the innermost periphery part and r=60 mm at the outermost periphery part. In addition, the iron core of the core No. c is a Unicore type wound core having a larger radius of curvature r (the radius of curvature r exceeds 5 mm) than the iron cores of the cores Nos. a, b, and d (Unicore type wound core), and the iron core of the core No. d is a Unicore type wound core having three bent portions 5 at one corner portion 3.

**[Table 1]**

| Core No. | Core shape | | | | | | |
|---|---|---|---|---|---|---|---|
| | L1 | L2 | L3 | L4 | L5 | r | φ |
| | mm | mm | mm | mm | mm | mm | ∘ |
| a | 197 | 66 | 47 | 152.4 | 4 | 1 | 45 |
| b | 197 | 66 | 47 | 152.4 | 4 | 5 | 45 |
| c | 197 | 66 | 47 | 152.4 | 4 | 6 | 45 |
| d | 197 | 66 | 47 | 152.4 | 4 | 2 | 30 |
| e | 197 | 66 | 47 | 152.4 | 4 | * | 90 |
| f | 197 | 66 | 47 | 152.4 | 4 | 2 | 45 |

Tables 2 to 5 show, based on various core shapes as described above, the average value (µm) of Ra(b) measured at 10 locations (measured at 10 fields of view) at the bent portion 5 described above, the average value (µm) of Ra(s) measured at 10 locations (measured at 10 fields of view) at the planar portion 4 (4a) described above, and the ratio Ra(b)/Ra(s) obtained by measuring 85 example materials in which the target bent angle ϕ(°), the steel sheet thickness (mm), and the tensile stress (MPa) applied in the longitudinal direction L were set, and the measured and evaluated iron core noise (dBA). Here, the above measurement at 10 locations means that, in the case of the bent portion 5, 10 steel sheets were arbitrarily extracted from one wound core, one location of each bent portion was set as one field of view, and Ra(b) and the measured bent angle were measured. The average heights Ra(b) and Ra(s) of the roughness curve element both are the average height Rc of the roughness curve element measured using a digital microscope (VHX-7000, commercially available from Keyence Corporation). The average height Rc of the roughness curve element was measured based on JIS B 0601 (2013). The cutoff values were λs=0 and λc=0, and vibration correction was performed for measurement. The measurement magnification was set to 500 to 700.

In evaluation of iron core noise, the above wound core was prepared and excited, and noise was measured. This noise measurement was performed in an anechoic chamber with a background noise of 16 dBA, a noise meter was installed at a position of 0.3 m from the surface of the iron core and the A characteristic was used as acoustic feeling correction. In addition, in the excitation, the frequency was set to 50 Hz, and the magnetic flux density was set to 1.7 T. An iron core noise of 44 dBA or less was determined to be satisfactory.

**[Table 2]**

| No | Cor e No. | Targe t bent angle ϕ (°) | Steel sheet thicknes s (mm) | Tensile stress (MPa) | Average of Ra(b) measure d at 10 locations on bent portion (µm) | Average of Ra(s) measure d at 10 locations on planar portion (µm) | Ratio Ra(b)/Ra( s) | Iron core noise (dBA ) |
|---|---|---|---|---|---|---|---|---|
| 1 | a | 45 | 0.23 | 0 | 6.68 | 0.78 | 8.56 | 47 |
| 2 | a | 45 | 0.23 | 1 | 6.53 | 0.78 | 8.37 | 46 |
| 3 | a | 45 | 0.23 | 2.5 | 6.03 | 0.77 | 7.83 | 48 |
| 4 | a | 45 | 0.23 | 3.5 | 6.04 | 0.76 | 7.95 | 47 |
| 5 | a | 45 | 0.23 | 3.8 | 5.04 | 0.76 | 6.63 | 46 |
| 6 | a | 45 | 0.23 | 4 | 3.75 | 0.75 | 5.00 | 36 |
| 7 | a | 45 | 0.23 | 6 | 3.55 | 0.76 | 4.67 | 35 |
| 8 | a | 45 | 0.23 | 9 | 3.44 | 0.78 | 4.41 | 32 |
| 9 | a | 45 | 0.23 | 10 | 3.24 | 0.75 | 4.32 | 33 |
| 10 | a | 45 | 0.23 | 11 | 3.02 | 0.77 | 3.92 | 27 |
| 11 | a | 45 | 0.23 | 13 | 2.95 | 0.78 | 3.78 | 26 |
| 12 | a | 45 | 0.23 | 14 | 2.56 | 0.77 | 3.32 | 35 |
| 13 | a | 45 | 0.23 | 15 | 1.43 | 0.75 | 1.91 | 36 |
| 14 | a | 45 | 0.23 | 16 | 0.77 | 0.77 | 1.00 | 37 |
| 15 | a | 45 | 0.23 | 17 | 0.74 | 0.77 | 0,96 | 45 |
| 16 | a | 45 | 0.23 | 20 | 0.62 | 0.77 | 0.81 | 47 |
| 17 | a | 45 | 0.23 | 30 | 0.63 | 0.78 | 0.81 | 46 |
| 18 | a | 45 | 0.23 | 45 | 0.53 | 0.78 | 0.68 | 46 |
| 19 | a | 45 | 0.23 | 65 | 0.44 | 0.77 | 0.57 | 52 |
| 20 | a | 45 | 0.23 | 10 (compressiv e stress) | 8.98 | 0.78 | 11.51 | 58 |

**[Table 3]**

| No | Cor e No. | Targe t bent angle ϕ (°) | Steel sheet thicknes s (mm) | Tensile stress (MPa) | Average of Ra(b) measure d at 10 location s on bent portion (µm) | Average of Ra(s) measure d at 10 location s on planar portion (µm) | Ratio Ra(b)/Ra( s) | Iron core noise (dBA ) |
|---|---|---|---|---|---|---|---|---|
| 21 | b | 45 | 0.23 | 0 | 6.61 | 0.78 | 8.48 | 48 |
| 22 | b | 45 | 0.23 | 1 | 6.46 | 0.78 | 8.29 | 47 |
| 23 | b | 45 | 0.23 | 2.5 | 5.97 | 0.77 | 7.75 | 49 |
| 24 | b | 45 | 0.23 | 3.5 | 5.98 | 0.76 | 7.87 | 48 |
| 25 | b | 45 | 0.23 | 3.8 | 4.99 | 0.76 | 6.57 | 47 |
| 26 | b | 45 | 0.23 | 4 | 3.75 | 0.75 | 5.00 | 37 |
| 27 | b | 45 | 0.23 | 6 | 3.51 | 0.76 | 4.62 | 36 |
| 28 | b | 45 | 0.23 | 9 | 3.41 | 0.78 | 4.37 | 33 |
| 29 | b | 45 | 0.23 | 10 | 3.21 | 0.75 | 4.28 | 34 |
| 30 | b | 45 | 0.23 | 11 | 0.78 | 0.77 | 1.01 | 28 |
| 31 | b | 45 | 0.23 | 13 | 0.78 | 0.78 | 1.00 | 27 |
| 32 | b | 45 | 0.23 | 14 | 2.53 | 0.77 | 3.29 | 36 |
| 33 | b | 45 | 0.23 | 15 | 1.42 | 0.75 | 1.89 | 37 |
| 34 | b | 45 | 0.23 | 16 | 3.85 | 0.77 | 5.00 | 38 |
| 35 | b | 45 | 0.23 | 17 | 0.73 | 0.77 | 0.95 | 46 |
| 36 | b | 45 | 0.23 | 20 | 0.61 | 0.77 | 0.80 | 48 |
| 37 | b | 45 | 0.23 | 30 | 0.62 | 0.78 | 0.80 | 47 |
| 38 | b | 45 | 0.23 | 45 | 0.52 | 0.78 | 0.67 | 47 |
| 39 | b | 45 | 0.23 | 65 | 0.44 | 0.77 | 0.57 | 53 |
| 40 | b | 45 | 0.23 | 10 (compressiv e stress) | 8.98 | 0.78 | 11.40 | 59 |
| 41 | b | 45 | 0.23 | 2.5 | 6.03 | 0.77 | 7.83 | 48 |

**[Table 4]**

| No | Cor e No. | Targe t bent angle ϕ (°) | Steel sheet thicknes s (mm) | Tensile stress (MPa) | Average of Ra(b) measure d at 10 location s on bent portion (µm) | Average of Ra(s) measure d at 10 location s on planar portion (µm) | Ratio Ra(b)/Ra( s) | Iron core noise (dBA ) |
|---|---|---|---|---|---|---|---|---|
| 42 | c | 45 | 0.23 | 30 | 0.58 | 0.78 | 0.74 | 48 |
| 43 | d | 30 | 0.23 | 1 | 6.53 | 0.78 | 8.37 | 49 |
| 44 | d | 30 | 0.23 | 4 | 3.75 | 0.75 | 5.00 | 36 |
| 45 | d | 30 | 0.23 | 10 | 0.98 | 0.75 | 1.31 | 33 |
| 46 | d | 30 | 0.23 | 16 | 3.85 | 0.77 | 5.00 | 37 |
| 47 | d | 30 | 0.23 | 45 | 6.34 | 0.78 | 8.13 | 51 |
| 48 | a | 45 | 0.15 | 0.1 | 7.33 | 0.76 | 9.64 | 52 |
| 49 | a | 45 | 0.15 | 4 | 3.85 | 0.77 | 5.00 | 36 |
| 50 | a | 45 | 0.15 | 16 | 0.77 | 0.77 | 1.00 | 37 |
| 51 | a | 45 | 0.18 | 0.3 | 6.28 | 0.77 | 8.16 | 48 |
| 52 | a | 45 | 0.18 | 4 | 3.67 | 0.77 | 4.77 | 37 |
| 53 | a | 45 | 0.18 | 10 | 1.02 | 0.77 | 1.32 | 28 |
| 54 | a | 45 | 0.18 | 24 | 0.61 | 0.77 | 0.79 | 56 |
| 55 | a | 45 | 0.2 | 0.4 | 6.89 | 0.77 | 8.95 | 51 |
| 56 | a | 45 | 0.2 | 7 | 1.04 | 0.77 | 1.35 | 26 |
| 57 | a | 45 | 0.2 | 5 (compressiv e stress) | 12.56 | 0.77 | 16.31 | 62 |
| 58 | a | 45 | 0.27 | 0.5 | 7.44 | 0.78 | 9.54 | 50 |
| 59 | a | 45 | 0.27 | 4 | 3.85 | 0.77 | 5.00 | 37 |
| 60 | a | 45 | 0.27 | 11 | 1.10 | 0.77 | 1.43 | 28 |
| 61 | a | 45 | 0.27 | 21 | 0.66 | 0.77 | 0.86 | 52 |
| 62 | a | 45 | 0.3 | 9 | 1.07 | 0.77 | 1.39 | 30 |

**[Table 5]**

| No | Cor e No. | Targe t bent angle ϕ (°) | Steel sheet thicknes s (mm) | Tensile stress (MPa) | Average of Ra(b) measure d at 10 location s on bent portion (µm) | Average of Ra(s) measure d at 10 location s on planar portion (µm) | Ratio Ra(b)/Ra( s) | Iron core noise (dBA ) |
|---|---|---|---|---|---|---|---|---|
| 63 | a | 45 | 0.35 | 10 | 1.08 | 0.78 | 1.38 | 31 |
| 64 | a | 45 | 0.35 | 30 | 0.49 | 0.78 | 0.63 | 54 |
| 65 | a | 45 | 0.35 | 2 (compressiv e stress) | 10.30 | 0.76 | 13.55 | 58 |
| 66 | e | 90 | 0.23 | 2.5 | 6.03 | 0.77 | 7.83 | 48 |
| 67 | e | 90 | 0.23 | 6 | 2.44 | 0.76 | 3.21 | 51 |
| 68 | e | 90 | 0.23 | 11 | 0.78 | 0.77 | 1.01 | 49 |
| 69 | e | 90 | 0.23 | 16 | 3.85 | 0.77 | 5.00 | 52 |
| 70 | c | 45 | 0.23 | 3 | 7.47 | 0.78 | 9.58 | 52 |
| 71 | c | 45 | 0.23 | 4 | 0.92 | 0.76 | 1.21 | 43 |
| 72 | c | 45 | 0.23 | 6 | 1.26 | 0.77 | 1.64 | 41 |
| 73 | c | 45 | 0.23 | 12 | 2.67 | 0.78 | 3.42 | 39 |
| 74 | c | 45 | 0.23 | 16 | 3.85 | 0.78 | 4.94 | 38 |
| 75 | c | 45 | 0.23 | 20 | 6.13 | 0.78 | 7.86 | 53 |
| 76 | a | 45 | 0.2 | 17 | 0.75 | 0.76 | 0.99 | 46 |
| 77 | a | 45 | 0.27 | 3 | 3.79 | 0.76 | 4.99 | 37 |
| 78 | f | 45 | 0.23 | 3 | 7.51 | 0.78 | 9.63 | 54 |
| 79 | f | 45 | 0.23 | 4 | 0.92 | 0.76 | 1.21 | 44 |
| 80 | f | 45 | 0.23 | 6 | 1.28 | 0.77 | 1.66 | 40 |
| 81 | f | 45 | 0.2 | 12 | 2.67 | 0.78 | 3.42 | 39 |
| 82 | f | 45 | 0.2 | 16 | 3.82 | 0.78 | 4.90 | 38 |
| 83 | f | 45 | 0.18 | 20 | 6.11 | 0.78 | 7.83 | 53 |
| 84 | f | 45 | 0.18 | 17 | 0.75 | 0.76 | 0.99 | 46 |
| 85 | f | 45 | 0.18 | 3 | 3.79 | 0.76 | 4.99 | 37 |

As can be understood from Tables 2 to 5, regarding the iron cores of the cores Nos. a, b, c, d, and f forming a Unicore type, if the steel sheet thickness was within a range of 0.15 mm to 0.35 mm, regardless of the sheet thickness, a tensile stress (tension) within a range of 4 MPa or more and 16 MPa or less was applied in the longitudinal direction L, and thus a ratio Ra(b)/Ra(s) satisfying the relationship of 1.00<Ra(b)/Ra(s)≤5.00 was obtained. Accordingly, the iron core noise was reduced to 44 dBA or less. On the other hand, if the tensile stress was too strong, the surface roughness became small, but there was a tendency for noise to deteriorate at that time due to strain or the like. In addition, the iron cores of the cores Nos. a, b, and c having a small radius of curvature r (5 mm or less) of the bent portion have iron core noise that was reduced more than the iron core of the core No. c with a radius of curvature of 6 mm. In addition, in the case of the iron core of the core No. e forming a trunk core type, when a tensile stress within a range of 4 MPa or more and 16 MPa or less was applied in the longitudinal direction L, even if the relationship of 1.00<Ra(b)/Ra(s)≤5.00 was satisfied, iron core noise could not be sufficiently reduced.

Based on the above results, it can be clearly understood that, in the wound core of the present invention, since the relationship of 1.00<Ra(b)/Ra(s)≤5.00 was satisfied when bending was performed while tensile stress was applied to the entire end surface (C cross section) of the steel sheet to be bent in the longitudinal direction, noise caused by plastic deformation strain was reduced.

### [Brief Description of the Reference Symbols]

1 Grain-oriented electrical steel sheet
4, 4a Planar portion
5 Bent portion
10 Wound core (wound core main body)
50 Device
70 Production device
71 Bending unit
72 Assembly unit

## Claims

1. A wound core (10) including a portion in which grain-oriented electrical steel sheets (1), in which planar portions (4, 4a) and bent portions (5) are alternately continuous in a longitudinal direction (L), are stacked in a sheet thickness direction (C) and are formed by stacking the grain-oriented electrical steel sheets (1) that have been individually bent in layers and assembled into a wound shape,
wherein, when an average height of a roughness curve element in a width direction (C) intersecting the longitudinal direction (L) forming a surface of the bent portion (5) of the grain-oriented electrical steel (1) sheet is Ra(b), and an average height of the roughness curve element in the width direction (C) forming a surface of the planar portion (4, 4a) of the grain-oriented electrical steel sheet (1) is Ra(s), the relationship of 1.00<Ra(b)/Ra(s)≤5.00 is satisfied.

2. The wound core (10) according to claim 1,
wherein the bent portion (5) has a radius of curvature of 1 mm or more and 5 mm or less.

3. A method of producing a wound core (10), comprising:
a bending process in which grain-oriented electrical steel sheets (1) are individually bent; and
an assembling process in which the bent grain-oriented electrical steel sheets (1) are stacked in layers and assembled into a wound shape to form a wound core (10) having a wound shape including a portion, in which grain-oriented electrical steel sheets (1) in which planar portions (4, 4a) and bent portions (5) are alternately continuous in a longitudinal direction (L), are stacked in a sheet thickness direction (C),
wherein, in the bending process, the grain-oriented electrical steel sheet is (1) bent while a tensile stress in a range of 4 MPa or more and 16 MPa or less is applied to the grain-oriented electrical steel sheet (1) in the longitudinal direction (L), whereby the relationship as defined in claim 1 is satisfied.

4. The method of producing a wound core (10) according to claim 3,
wherein, in the bending process, the grain-oriented electrical steel sheet (1) is bent so that the radius of curvature of the bent portion (5) of the grain-oriented electrical steel sheet (1) is 1 mm or more and 5 mm or less.

5. A wound core production device (70), comprising:
a bending unit (71) that individually bends grain-oriented electrical steel sheets (1); and
an assembly unit (72) that stacks the bent grain-oriented electrical steel sheets (1) in layers and assembles them into a wound shape to form a wound core (10) having a wound shape including a portion in which grain-oriented electrical steel sheets (1), in which planar portions (4, 4a) and bent portions (5) are alternately continuous in a longitudinal direction (L), are stacked in a sheet thickness direction (C),
wherein the bending unit (71) bends the grain-oriented electrical steel sheet (1) while applying a tensile stress in a range of 4 MPa or more and 16 MPa or less to the grain-oriented electrical steel sheet (1) in the longitudinal direction (L), whereby the relationship as defined in claim 1 is satisfied.

6. The wound core production device (70) according to claim 5,
wherein the bending unit (71) bends the grain-oriented electrical steel sheet (1) so that the radius of curvature of the bent portion (5) of the grain-oriented electrical steel sheet (1) is 1 mm or more and 5 mm or less.

## Patentansprüche

1. Ein gewickelter Kern (10), der einen Abschnitt beinhaltet, in dem kornorientierte Elektrostahlbleche (1), bei denen ebene Abschnitte (4, 4a) und gebogene Abschnitte (5) in einer Längsrichtung (L) abwechselnd durchgehend sind, in einer Blechdickenrichtung (C) gestapelt sind und durch Stapeln der kornorientierten Elektrostahlbleche (1) gebildet sind, die einzeln in Schichten gebogen und in eine gewickelte Form gebracht wurden,
wobei, wenn eine mittlere Höhe eines Elements einer Rauheitskurve in einer Breitenrichtung (C), die die Längsrichtung (L) schneidet, die eine Oberfläche des gebogenen Abschnitts (5) des kornorientierten Elektrostahlblechs (1) bildet, Ra(b) ist, und eine mittlere Höhe des Elements der Rauheitskurve in die Breitenrichtung (C), die eine Oberfläche des ebenen Abschnitts (4, 4a) des kornorientierten Elektrostahlblechs (1) bildet, Ra(s) ist, die Beziehung 1,00 < Ra(b)/Ra(s) ≤ 5,00 erfüllt ist.

2. Der gewickelte Kern (10) gemäß Anspruch 1,
wobei der gebogene Abschnitt (5) einen Krümmungsradius von 1 mm oder mehr und 5 mm oder weniger aufweist.

3. Ein Verfahren zur Herstellung eines gewickelten Kerns (10), umfassend:
ein Biegeverfahren, in dem kornorientierte Elektrostahlbleche (1) einzeln gebogen werden; und
ein Montageverfahren, in dem die gebogenen kornorientierten Elektrostahlbleche (1) in Schichten gestapelt und in eine gewickelte Form gebracht werden, um einen gewickelten Kern (10) mit einer gewickelten Form zu bilden, der einen Abschnitt beinhaltet, in dem kornorientierte Elektrostahlbleche (1), bei denen ebene Abschnitte (4, 4a) und gebogene Abschnitte (5) in einer Längsrichtung (L) abwechselnd durchgehend sind, in einer Blechdickenrichtung (C) gestapelt sind,
wobei in dem Biegeverfahren das kornorientierte Elektrostahlblech (1) gebogen wird, während eine Zugspannung in einem Bereich von 4 MPa oder mehr und 16 MPa oder weniger auf das kornorientierte Elektrostahlblech (1) in der Längsrichtung (L) ausgeübt wird, wodurch die in Anspruch 1 definierte Beziehung erfüllt wird.

4. Das Verfahren zur Herstellung eines gewickelten Kerns (10) gemäß Anspruch 3, wobei das kornorientierte Elektrostahlblech (1) in dem Biegeverfahren gebogen wird, so dass der Krümmungsradius des gebogenen Abschnitts (5) des kornorientierten Elektrostahlblechs (1) 1 mm oder mehr und 5 mm oder weniger beträgt.

5. Eine Vorrichtung zur Herstellung eines gewickelten Kerns (70), umfassend:
eine Biegeeinheit (71), die kornorientierte Elektrostahlbleche (1) einzeln biegt; und
eine Montageeinheit (72), die die gebogenen kornorientierten Elektrostahlbleche (1) in Schichten stapelt und sie in eine gewickelte Form bringt, um einen gewickelten Kern (10) mit einer gewickelten Form zu bilden, der einen Abschnitt beinhaltet, in dem kornorientierte Elektrostahlbleche (1), bei denen ebene Abschnitte (4, 4a) und gebogene Abschnitte (5) in einer Längsrichtung (L) abwechselnd durchgehend sind, in einer Blechdickenrichtung (C) gestapelt sind,
wobei die Biegeeinheit (71) das kornorientierte Elektrostahlblech (1) biegt, während eine Zugspannung in einem Bereich von 4 MPa oder mehr und 16 MPa oder weniger auf das kornorientierte Elektrostahlblech (1) in der Längsrichtung (L) ausgeübt wird, wodurch die in Anspruch 1 definierte Beziehung erfüllt wird.

6. Die Vorrichtung zur Herstellung eines gewickelten Kerns (70) gemäß Anspruch 5,
wobei die Biegeeinheit (71) das kornorientierte Elektrostahlblech (1) biegt, so dass der Krümmungsradius des gebogenen Abschnitts (5) des kornorientierten Elektrostahlblechs (1) 1 mm oder mehr und 5 mm oder weniger beträgt.

## Revendications

1. Noyau enroulé (10) comprenant une portion dans laquelle des tôles d'acier électrique à grains orientés (1), dans lesquelles des portions planes (4, 4a) et des portions cintrées (5) sont continues en alternance dans la direction longitudinale (L), sont empilées dans la direction de l'épaisseur des tôles (C) et sont formées par empilement des tôles d'acier électrique à grains orientés (1) qui ont été individuellement cintrées en couches et assemblées sous une forme enroulée,
dans lequel, quand la hauteur moyenne d'un élément de courbe de rugosité dans la direction de la largeur (C) croisant la direction longitudinale (L) formant une surface de la portion cintrée (5) de la tôle d'acier électrique à grains orientés (1) est Ra(b), et la hauteur moyenne de l'élément de courbe de rugosité dans la direction de la largeur (C) formant une surface de la portion plane (4, 4a) de la tôle d'acier électrique à grains orientés (1) est Ra(s), la relation 1,00 < Ra(b)/Ra(s) ≤ 5,00 est satisfaite.

2. Noyau enroulé (10) selon la revendication 1
dans lequel la portion cintrée (5) a un rayon de courbure de 1 mm ou plus et 5 mm ou moins.

3. Méthode de production d'un noyau enroulé (10), comprenant :
un procédé de cintrage dans lequel des tôles d'acier électrique à grains orientés (1) sont individuellement cintrées ; et
un procédé d'assemblage dans lequel les tôles d'acier électrique à grains orientés (1) sont empilées en couches et assemblées sous une forme enroulée pour former un noyau enroulé (10) ayant une forme enroulée comprenant une portion, dans laquelle des tôles d'acier électrique à grains orientés (1) dans lesquelles des portions planes (4, 4a) et des portions cintrées (5) sont continues en alternance dans la direction longitudinale (L), sont empilées dans la direction de l'épaisseur des tôles (C),
dans laquelle, dans le procédé de cintrage, la tôle d'acier électrique à grains orientés (1) est cintrée tandis qu'une contrainte de traction située dans la plage allant de 4 MPa ou plus à 16 MPa ou moins est appliquée à la tôle d'acier électrique à grains orientés (1) dans la direction longitudinale (L), moyennant quoi la relation telle que définie dans la revendication 1 est satisfaite.

4. Méthode de production d'un noyau enroulé (10) selon la revendication 3,
dans laquelle, dans le procédé de cintrage, la tôle d'acier électrique à grains orientés (1) est cintrée de façon que le rayon de courbure de la portion cintrée (5) de la tôle d'acier électrique à grains orientés (1) soit de 1 mm ou plus et 5 mm ou moins.

5. Dispositif de production de noyau enroulé (70), comprenant :
une unité de cintrage (71) qui cintre individuellement des tôles d'acier électrique à grains orientés (1) ; et
une unité d'assemblage (72) qui empile les tôles d'acier électrique à grains orientés (1) en couches et les assemble sous une forme enroulée pour former un noyau enroulé (10) ayant une forme enroulée comprenant une portion dans laquelle des tôles d'acier électrique à grains orientés (1), dans lesquelles des portions planes (4, 4a) et des portions cintrées (5) sont continues en alternance dans la direction longitudinale (L), sont empilées dans la direction de l'épaisseur des tôles (C),
dans lequel l'unité de cintrage (71) cintre la tôle d'acier électrique à grains orientés (1) tout en appliquant une contrainte de traction située dans la plage allant de 4 MPa ou plus à 16 MPa ou moins à la tôle d'acier électrique à grains orientés (1) dans la direction longitudinale (L), moyennant quoi la relation telle que définie dans la revendication 1 est satisfaite.

6. Dispositif de production de noyau enroulé (70) selon la revendication 5,
dans lequel l'unité de cintrage (71) cintre la tôle d'acier électrique à grains orientés (1) de façon que le rayon de courbure de la portion cintrée (5) de la tôle d'acier électrique à grains orientés (1) soit de 1 mm ou plus et 5 mm ou moins.
